

Jan. 15, 1952

P. TORCHET

2,582,661

METHOD FOR ELECTROLYTICALLY REFINING ALUMINUM

Filed July 19, 1946



INVENTOR:

PIERRE TORCHET

By Wenderoth, Suid +  
Poncale

ATTORNEYS

## UNITED STATES PATENT OFFICE

2,582,661

METHOD FOR ELECTROLYTICALLY  
REFINING ALUMINUM

Pierre Torchet, Verneuil-sur-Seine, France, assignor to Pechiney-Compagnie de Produits Chimiques et Electrometallurgiques, a French society

Application July 19, 1946, Serial No. 684,671  
In France December 3, 1945

6 Claims. (Cl. 204—67)

1

The object of my invention is to recover in a state of great purity the aluminium contained in the scrap of certain alloys of said metal, by adapting to said operation the method disclosed in the U. S. Patent No. 2,034,339 dated March 17, 1936, for the refining of aluminium.

According to this method, there are superposed in the molten state inside an electrolytic vat a layer of heavy aluminium alloy serving as an anode and a layer of a selective molten electrolyte over which the refined aluminium forming at the cathode floats.

The electrolyte comprises a mixture of aluminium fluoride, sodium fluoride and an alkaline-earth chloride, the ratio of the amount of aluminium fluoride to that of sodium fluoride being greater than the corresponding ratio of the same bodies in cryolite, the mixture having a melting point between 700° C. and 800° C.

If the heavy component of the anodic alloy or bottom alloy is copper, this alloy should contain at least 28% of copper for its density to be sufficient. Its copper contents should not on the other hand rise beyond 40% without detrimentally affecting the purity of the aluminium produced at the cathode.

During the electrolysis, the impurities of the raw aluminium accumulate inside the alloy at the bottom of the vat. As soon as the content of copper in said alloy reaches a value near its upper limit, it is admixed with aluminium in order to lower the contents of copper. As a matter of fact, when refining aluminium, the level of the lower alloy mass varies but little in practice, for instance between 17 and 20 cms. above the bottom of a vat of 3 square meters because the contents of iron in said alloy also increase and when they reach too considerable a value, the alloy becomes pasty. It is therefore necessary to remove the alloy and to replace it by a further load with low contents of iron. This operation is delicate and costly; the reason thereof is that even with the greatest care, the electrolytic vat has to operate during 6 to 10 days before it is possible to obtain again at the cathode refined aluminium of a high grade of purity.

Particular difficulties are met with if instead of refining aluminium, it is desired to obtain through the same means refined aluminium, starting from an alloy such as Duralumin for instance containing:

Al 93.7% Cu 4% — Mg 0.7% —

Mn 0.6% — Si 0.5% — Fe 0.5%

The magnesium contained in the Duralumin

would also be a source of trouble because it would attack the electrolysing bath, but it is also easy to eliminate same by previously melting the Duralumin in presence of a salt such as cryolite, for instance, in the usual manner. The alloy from which the magnesium has been removed has substantially the same contents of copper as the original alloy.

If it is desired to extract aluminium in a state of high purity through the above disclosed method i. e. with a volume of lower alloy layer varying between very narrow limits, the contents of copper of said alloy reach rapidly the maximum value allowable before even the contents of iron become troublesome. It is therefore necessary to often renew the alloy, say about every 30 days. As during the 6 or 10 days following this renewal the aluminium produced does not reach the high grade of purity desired, this metal of exceptional quality is obtained only during 20 to 24 days out of 30 which renders the purification of scrap Duralumin through this method of very small economical interest.

The present invention corrects such disadvantages by permitting elongating considerably the lapse of time during which the metal of highest purity is obtained.

According to the present invention, the anodic layer receives, in addition to the amount of alloy to be treated corresponding to the refined aluminium produced at the cathode, an excess of said alloy such that while allowing a progressive increase of the depth of the lower alloy layer, the latter may retain copper contents which remain lower than the maximum value consistent with the purity of the refined aluminium obtained.

I form thus inside the anodic alloy layer an important reserve of copper which is removed periodically at long intervals and in large amounts. It is only necessary that the alloy to be treated diffuses rapidly enough in said lower layer when it is added.

It is possible to allow a variation in the depth of the lower alloy layer by starting from a value lower than that generally adopted in the refining of aluminium. It is only necessary that the alloy to be treated diffuses rapidly enough in said lower layer when it is added. Instead of a thickness of 17 to 20 centimeters as disclosed for the case of the refining of aluminium in a vat of 3 square meters it is possible to admit a minimum thickness of 10 to 12 centimeters for the lower alloy. As to the maximum thickness of said lower layer of alloy, it is limited in principle only by the con-

ditions of overflowing of the electrolysis vat. It is however preferable to limit the increase of the thickness of the lower alloy layer to a value which is at the utmost equal to the thickness of the electrolyte layer. In practice in the case of Duralumin, there is added daily to the anodic layer an excess of Duralumin of the magnitude of 2 to 4% with reference to the amount corresponding to the production of refined aluminium, the Duralumin being preliminarily freed from its magnesium by fusion in the presence of cryolite as indicated above.

Appended drawing shows by way of example a cross-sectional view passing centrally through an electrolysis vat adapted for use in the execution of the present invention.

In the drawings, 1 designates the body of the cell, 2 designates the current feeding means for the anodic blocks 3, said means passing through the bottom of the cell, 4 designates the lower alloy layer contacting with the blocks 3 while 5 designates the electrolyte layer over which floats the layer 6 of refined aluminium. Cathodic blocks are adapted to dip in the layer 6 carried by rods 8 adapted to be moved vertically through actuation of the hand wheel 9a. The latter is carried by a shaft 9 mounted on a gantry 10 mounted over the cell, said shaft 9 controlling the rods 8 through any suitable means.

The left hand side of the drawing shows the cell at the beginning of an operating period. The thickness  $h$  of the heavy alloy layer is then at its minimum value. Towards the end of the operating period as illustrated in the right hand part of the drawing, the respective thickness  $i$  of the electrolyte layer and  $j$  of the layer of refined aluminium have remained unaltered while the anodic alloy layer at the bottom of the vat has increased by a value substantially equal to the thickness of the electrolyte layer, so that its new thickness  $h'$  is more than twice  $h$ .

#### Examples

1. An electrolytic vat of 3 sq. meters bottom is used for the refining of aluminum; it is a vat of known type in which the thickness of the lower alloy layer, is usually kept between 17 and 20 cms., while aluminum is electrolytically refined in it by known processes.

A refining operation of aluminum is carried out with—at the start—a lower layer of alloy to be refined having the thickness of only 12 cms.; in the course of refining this layer is allowed to reach the thickness of 25 cms. i. e. to become about 2 times as thick as it was at the start of the operation. Then instead of being compelled to renew the anodic alloy after 30 days as would have been necessary if usual principles (thickness kept between 17 and 20 cms.) had been respected, it is possible to renew said anodic alloy layer only after 115 days. It is therefore possible to produce refined aluminum during 105 to 109 days out of 115.

In another operation the thickness of the lower alloy layer was of 10 cms. at the start and was allowed to reach, in the course of the refining, 30 cms., that means the anodic layer became 3 times as thick as it was, sufficient to renew the alloy every 180 days and aluminum was refined to a high grade of purity during 170 to 174 days out of 180.

The layer forming the anode is thus permitted to become 2 to 3 times as thick as it was at the refining operation.

2. In an electrolytic vat of 8 square meters, the

introduced lower alloy layer, at the start of the operation, is 10 cms. thick; said layer is allowed to grow to a thickness of 25 cms. It is possible under such conditions to renew the alloy only every 381 days so that it is possible to produce refined aluminium during 370 to 375 days out of 381. This provides a range of from 30 to 380 days for the renewal of the anodic layer.

The anodic alloy reaches its critical maximum contents of copper before it is saturated with iron. When the contents of copper of said alloy reach their upper limit, it is therefore possible to remove only a part of the alloy and to reduce the contents of copper of the remaining alloy down to the desired minimum value i. e. 28% through an addition of Duralumin.

The operation continues thus without it being necessary to incorporate copper as such into the bath as the copper introduced by the Duralumin is sufficient for the requirements.

The iron contents of the lower alloy increase progressively but have a tendency to reach a limit of 6% of which 5% are provided by the Duralumin and 1% by the operations inside the vat.

As a result 1000 kgs. of Duralumin from which the magnesium has been eliminated and containing: 945 kgs. of Al—40 kgs. of Cu—6 kgs. of Fe—5 kgs. of Si—6 kgs. of Mn produce 900 kgs. of refined aluminium and 100 kgs. of an alloy containing: Al 43%—Cu 40%—Fe 8%—Si 5%—Mn 6%—which latter alloy is eliminated.

The present invention is by no means limited in its application to Duralumin and it may be used with any aluminium alloys, wherein the proportions of alloyed metals are of comparable magnitude, which means containing more than 90% aluminium, provided their contents of iron do not lead to a more frequent replacement of the lower alloy. In particular it is perfectly applicable to alloys containing zinc, which latter metal may in fact replace wholly or partly copper in the anodic alloy.

What I claim is:

1. In a method for electrolytically refining aluminium, which comprises superposing in an electrolytic vat, a layer of molten aluminium alloy containing at least one heavy metal and free of magnesium forming the anode, a layer of melted electrolyte mixture of aluminium fluoride, sodium fluoride and an alkaline-earth chloride, the ratio of the amount of aluminium fluoride to that of sodium fluoride being greater than the corresponding ratio of the same bodies in cryolite, said electrolyte mixture having a melting point between 700° C. and 800° C., and a layer of aluminium forming the cathode, additions of aluminium to be refined to said layer forming the anode being made in the course of the refining operation, the steps consisting in daily adding to said molten alloy forming the anode an amount of alloy free of magnesium containing more than 90% of aluminium, greater than the amount of the same which includes the quantity of daily produced refined aluminium, and removing said layer forming the anode for renewing it only every 30 to 380 days.

2. In a method for electrolytically refining aluminium which comprises superposing in an electrolytic vat, a layer of molten aluminium alloy containing at least one heavy metal and free of magnesium forming the anode, a layer of melted electrolyte mixture of aluminium fluoride, sodium fluoride and an alkaline-earth chloride, the ratio of the amount of aluminium fluoride to that of

sodium fluoride being greater than the corresponding ratio of the same bodies in cryolite, said electrolyte mixture having a melting point between 700° C. and 800° C., and a layer of aluminium forming the cathode, additions of aluminium to be refined to said layer forming the anode being made in the course of the refining operation, the steps consisting in daily adding to said molten alloy forming the anode an amount of alloy free of magnesium containing more than 90% of aluminium, greater by 2 to 4% than the amount of the same which includes the quantity of daily produced refined aluminium, and removing said layer forming the anode for renewing it only every 30 to 380 days.

3. In a method for electrolytically refining aluminium, which comprises superposing in an electrolytic vat, a layer of molten aluminium alloy containing at least one heavy metal and free of magnesium forming the anode, a layer of melted electrolyte mixture of aluminium fluoride, sodium fluoride and an alkaline-earth chloride, the ratio of the amount of aluminium fluoride to that of sodium fluoride being greater than the corresponding ratio of the same bodies in cryolite, said electrolyte mixture having a melting point between 700° C. and 800° C., and a layer of aluminium forming the cathode, additions of aluminium to be refined to said layer forming the anode being made in the course of the refining operations, the steps consisting in daily adding to said molten alloy forming the anode an amount of alloy free of magnesium containing more than 90% of aluminium, greater than the amount of the same which includes the quantity of daily produced refined aluminium, and removing said layer forming the anode for renewing it only every 30 to 380 days, when said layer forming the anode becomes 2 to 3 times as thick as it is at the start of the refining operation.

4. In a method for electrolytically refining aluminium which comprises superposing in an electrolytic vat, a layer of molten aluminium alloy containing at least one heavy metal and free of

magnesium forming the anode, a layer of melted electrolyte mixture of aluminium fluoride, sodium fluoride and an alkaline-earth chloride, the ratio of the amount of aluminium fluoride to that of sodium fluoride being greater than the corresponding ratio of the same bodies in cryolite, said electrolyte mixture having a melting point between 700° C. and 800° C., and a layer of aluminium forming the cathode, additions of aluminium to be refined to said layer forming the anode being made in the course of the refining operation, the steps consisting in daily adding to said molten alloy forming the anode an amount of alloy free of magnesium containing more than 90% of aluminium, greater by 2 to 4% than the amount of the same which includes the quantity of daily produced refined aluminium, and removing said layer forming the anode for renewing it only every 30 to 380 days, when said layer forming the anode becomes 2 to 3 times as thick as it is at the start of the refining operation.

5. The method claimed in claim 1 where the thickness of the said layer forming the anode is of 10 to 12 centimeters at the start of the refining operation and when it reaches 25 to 30 centimeters said layer is removed and renewed.

6. The method claimed in claim 2 where the thickness of said layer forming the anode is of 10 to 12 centimeters at the start of the refining operation and when it reaches 25 to 30 centimeters said layer is removed and renewed.

PIERRE TORCHET.

#### REFERENCES CITED

35 The following references are of record in the file of this patent:

#### UNITED STATES PATENTS

| Number       | Name   | Date          |
|--------------|--------|---------------|
| 40 1,534,317 | Hoopes | Apr. 21, 1925 |
| 1,534,318    | Hoopes | Apr. 24, 1925 |
| 1,782,616    | Hulin  | Nov. 25, 1930 |
| 2,034,339    | Gadeau | Mar. 19, 1936 |